

Oct. 11, 1938.

P. HART ET AL

2,132,734

LAUNDRY NET

Filed Aug. 19, 1936



Fig. 1



Fig. 2



Fig. 4



Fig. 3

INVENTORS

BY Parker Hart  
Robert W. Hart Jr.  
Richard Whiting  
ATTORNEY

## UNITED STATES PATENT OFFICE

2,132,734

## LAUNDRY NET

Parker Hart, Rye, N. Y., and Robert W. Hart, Jr.,  
Cambridge, Mass.

Application August 19, 1936, Serial No. 96,712

6 Claims. (Cl. 28—1)

This invention relates to laundry nets or bags of the open mesh type commonly employed in laundries to confine the washing of the individual customer during the laundering processes, and it is particularly directed to a novel construction of the yarns or cords of such bags adapted to resist the deleterious action on the bags of the washing and bleaching solutions into which the bags are immersed.

10 It is the common practice of laundries to enclose the washing of each customer in an individual open mesh bag and to launder the articles within the bag by immersing the bag in various cleansing and bleaching solutions, the interstices of the bag being sufficiently large to permit circulation of the fluids therethrough to launder the articles within the bag. Bags of this character have commonly been woven of cotton cords and the chemical and physical actions of the laundering solutions on these strands have caused rapid deterioration of the bags. The absorption of liquid by the cords causes them to swell and thereby to become weakened; the moist cords shrink, thereby reducing the capacity of the bag; 25 and the absorbed moisture causes the cords to rot, to mildew and to become sour and give off unpleasant odors. The action of the washing and bleaching fluids on the cords is also partly chemical in nature in that the basic washing fluids, the acidic "sour" rinses, and the oxidizing bleaches react chemically on the cord fibres and cause them to deteriorate rapidly.

It is an object of this invention to provide a bag of this character which lasts considerably longer than those now in commercial use and which neither shrinks nor becomes offensive during use. To that end we have found that by impregnating the fibrous cords of the bag, preferably after they have been woven into bag form, but also, if desired, before weaving, with a rubber composition preferably of certain characteristics noted in detail hereafter, we can effectively prevent, or at least materially reduce, both absorption of fluids by the cords and the chemical action of the fluids on the cords and we can thereby eliminate the above noted effects of such absorption and chemical action.

These and further objects and advantages of our invention will appear from a more detailed description thereof, in connection with the accompanying drawing, in which:

Fig. 1 is a perspective view of a laundry bag of the type above identified;

Fig. 2, on a larger scale than Fig. 1, shows the open weave of such laundry bags and indicates

the cords as having been treated in accordance with our invention;

Fig. 3 is a perspective view, on a greatly enlarged scale, of one of the treated cords, and

Fig. 4 is a cross-sectional view of such a cord indicating the manner in which the rubberizing material penetrates to the interior of the cord.

Referring to the drawing and particularly to Fig. 1, we have indicated at 1 a laundry bag made in any suitable way, such as by being woven on a circular loom if a continuous side wall without seam is desired. The bottom of the bag is formed with the usual ribbing 2 and may be closed by stitching. The top is closed after receiving the articles to be laundered, by being gathered together and pinned with a large safety pin as indicated at 3.

Fig. 2 illustrates the coarseness of the weave of such bags, the weft or filling threads 4 being widely separated from each other and the warp threads 5 being similarly spaced to provide large apertures 6 through which the washing fluids may gain access to, and circulate through, the clothing within. The size of the interstices 6 may well vary to suit the requirements of the individual user of such bags, as may the style of weave, but Fig. 2 illustrates in full scale a webbing of a popular size and style.

As shown in Fig. 3, the cords 10, constituting both the warps 5 and wefts 4, are quite coarse for the sake of durability, and may be constructed of a large number of plies 11 of yarn suitably spun or twisted to form the cording 10.

After the bag has been woven from cords of this character, we process the bag by first immersing it in a bath comprising a rubber solution or dispersion preferably containing elements which render the rubber capable of subsequent vulcanization and produce a deposited vulcanized rubber which resists abrasion and chemical action by the acids, bases and oxidizing agents to which the bag is exposed during use.

As an example of a bath which we have found particularly well adapted for the purpose, we employ a gasoline solution of the following materials, the solution containing about 15% solids:

|                       | Per cent    |
|-----------------------|-------------|
| Smoked sheet rubber   | 40          |
| Lithopone             | 35          |
| Paris white           | 22.15       |
| Lime                  | 50          |
|                       | 1.25        |
|                       | (or higher) |
| Sulphur               | .80         |
| Stearic acid          | .40         |
| Mercaptobenzothiazole | .40         |
|                       | 55          |

After the bag has been immersed in the above solution for a suitable period of time, such as a minimum of approximately two minutes, it is removed and dried to evaporate any gasoline which may cling to the cords. The dried bag is then subjected to heat treatment with live steam at approximately 40 lbs. pressure for forty-five minutes. It is then removed and washed in cold water to remove any possible traces of iron oxide which may have been deposited during the steaming treatment. The bag is then ready for use.

As illustrated in Figs. 3 and 4, the cords 10 so treated are impregnated with rubber which penetrates the individual strands 11 of the cord 15 and also embeds them in a surrounding sheath of rubber as indicated at 20. This penetration is effected partly by the steam treatment. The outside of the cord 10 is coated with rubber as indicated at 21.

We have found that in use, a bag so constructed and treated will not only be impervious to water and resistant to acids and oxidizing agents of the character commonly employed in laundries, but, furthermore, the rubber itself has abrasive 25 resisting qualities and it thereby protects the cords against wear. The vulcanization of the rubber strengthens it and removes most of its natural tackiness. The lime is effective to counteract the acids in the "sour" rinsing solutions 30 and prevents the rubber from becoming tacky as a result of such acidity.

In a similar manner webbing of any sort, such as tennis nets and the like, may be rendered substantially impervious to moisture or mild chemical fluids.

We do not wish to limit ourselves to the specific rubber formula set forth above, as other suitable formulae will present themselves to the man skilled in the art. For example, a rubber dispersion, aqueous if desired, such as latex, may be employed in place of a gasoline or similar solution as noted above.

While our preferred method is to treat the cords after they have been woven or otherwise concatenated into bag form, the cords can be treated prior to fabrication with good results.

In that event we prefer to dip the cords into a solution of the type above specified and after steam treating the cords to vulcanize the rubber thus deposited, in the manner above described, we then dip the cords in a latex dispersion and then pass them between circumferentially grooved rollers to smooth the deposited coating.

Our invention is not to be limited to the above details except as indicated in the appended claims.

We claim:

1. As an article of manufacture, a laundry bag 5 of the character described, constructed of fibrous cords concatenated to present open meshes for the circulation of laundry fluids through articles within the bag, the said fibrous cords being impregnated with a material which renders them 10 substantially impervious to said fluids.

2. As an article of manufacture, a laundry bag 15 of the character described, constructed of fibrous cords concatenated to present open meshes for the circulation of laundry fluids through articles 20 within the bag, each of said cords comprising a plurality of fibrous plies twisted together, each of said plies being impregnated with and incased in a material which renders the cord substantially impervious to said fluids.

3. As an article of manufacture, a laundry bag 25 of the character described, constructed of fibrous cords concatenated to present open meshes for the circulation of laundry fluids through articles within the bag, each of said cords comprising a plurality of fibrous plies twisted together, each of said plies being impregnated with and incased in a rubberizing material and the cords so constructed each being 30 enclosed in a protective sheath of rubberizing material whereby to render the cords substantially impervious to said fluids.

4. As an article of manufacture, a laundry bag 35 of the character described, constructed of fibrous cords concatenated to present open meshes for the circulation of laundry fluids through articles within the bag, the said cords being impregnated with vulcanized rubber which renders them substantially impervious to water and the said vulcanized rubber being slightly basic to counteract 40 the acidity of the washing fluids.

5. As an article of manufacture, a laundry bag 45 of the character defined in claim 1, in which the said material with which the fibrous cords are impregnated is a rubberizing material.

6. As an article of manufacture, a laundry bag 50 of the character defined in claim 1, in which the said material with which the fibrous cords are impregnated is slightly basic to counteract the acidity of the washing fluids.

PARKER HART.  
ROBERT W. HART, JR.